

Oct. 13, 1925.

1,556,642

W. H. SMITH

PROCESS OF CASTING MALLEABLE CASTINGS

Filed April 10, 1924



Fig. 1.



Fig. 2.



Fig. 3.



Fig. 4.

Inventor

William H. Smith,

By *Robert H. Smith*

Attorneys

Patented Oct. 13, 1925.

1,556,642

# UNITED STATES PATENT OFFICE.

WILLIAM H. SMITH, OF DEARBORN, MICHIGAN, ASSIGNOR TO FORD MOTOR COMPANY,  
OF DETROIT, MICHIGAN, A CORPORATION OF DELAWARE.

## PROCESS OF CASTING MALLEABLE CASTINGS.

Application filed April 10, 1924. Serial No. 705,409.

To all whom it may concern:

Be it known that I, WILLIAM H. SMITH, a citizen of the United States, residing at Dearborn, in the county of Wayne and State 5 of Michigan, have invented certain new and useful Improvements in Processes of Casting Malleable Castings, of which the following is a specification, reference being had therein to the accompanying drawings.

10 Malleable gray iron castings when cast in metallic molds or dies, are first white iron, or chilled cast iron, and the combined carbon is then converted by special heat treatment into an uncombined, amorphous 15 condition, which treatment renders the castings malleable.

The usual method of producing die cast iron castings is to produce white iron castings which are then annealed at a high temperature, causing a conversion of the carbon 20 content to an amorphous, uncombined condition, the castings being permitted to slowly cool. Essential conditions are proper control of temperature and time, the cooling 25 being sufficiently delayed to give proper annealing. The texture on malleability of castings cast in dies, is dependent upon the rate of temperature drop through the critical range of cooling, which is about 1200° F.

30 The common practice involves several independent steps and separate annealing and handling, with difficulty arising from inaccurate control of time and temperature of cooling, oxidization, and required skill in 35 producing a uniform product.

This invention relates to a process or method for producing malleable gray iron castings, and its object is to simplify methods, increase production, insure uniform 40 product, and provide certain other new and useful features, all as hereinafter more fully described, the invention consisting in providing a method wherein the operation of cooling the metal to give the desired malleability is introduced into the casting operation and accurately controlled as to time and temperature by controlling the transfer of heat from casting to cooling medium, and further consists in certain other new and 45 useful features, all as hereinafter more fully described, reference being had to the accompanying drawing illustrative of one means whereby the method embodying the 50 invention may be performed.

55 In the drawing,

Figure 1 is a plan view of a mold construction shown for the purpose of illustrating the method embodying the invention;

Fig. 2 is a longitudinal vertical section through the same;

Fig. 3 is a transverse section substantially upon the line 3—3 of Fig. 2, and

Fig. 4 is a sectional perspective detail of a casting cast in the mold.

The present invention contemplates the 65 casting of molten iron in a metallic mold or die, the temperature of which is raised to a proper degree of heat above 500° F. and maintained at such temperature by a suitable heat conducting fluid to maintain a temper- 70 ature equilibrium between the metal and said heating medium, whereby the proper time in the fall of the temperature of the casting is secured to produce malleability of the casting.

Formerly it has been deemed necessary to cast the metal and then reheat the casting to anneal the iron and produce malleability. The present invention contemplates the casting 75 of the metal in dies and controlling the temperature of these dies to regulate the rate of cooling of the cast metal and produce malleability thereof.

As illustrative of a die construction which may be employed in the carrying out of the 80 present method or process, a two part die formed of a suitable material, preferably metal, is provided, the confronting faces of which parts are formed to give the desired configuration to the casting. These two 85 parts 1 and 2 of the die or mold preferably together form a wall 4 which separates chambers 3, each die part forming a part of said wall and the chambers forming receptacles or passages for a fluid body 5 which is thus 90 in direct contact with the die or mold wall. The fluid is maintained, in any suitable manner, at the proper temperature to maintain a certain heat ratio between die walls and metal introduced into the dies, the 95 temperature of the metal casting being gradually reduced at the proper rate, by convection, so that the desired malleability 100 of the casting 9 will take place within the dies, and when discharged, the casting will 105 have the desired structure without higher heating. This fluid which may be maintained at a uniform high temperature by the heat transferred thereto by the molten metal in casting or otherwise, may be cir- 110

- culated in any suitable manner if found desirable, to gradually carry off the heat imparted thereto by the metal through the walls of the die.
- 5 In the present instance and as illustrated in the accompanying drawing, the dies are cooled and at the same time maintained at the proper temperature to prevent too rapid cooling of the casting, by maintaining a body 10 of molten tin at a temperature of 500° F. or over and in direct contact with the walls 4 of the metallic die which walls form the two parts of the die or mold proper, between which the casting is formed. As tin is one 15 of the metals having a high heat conductivity and which can be maintained fluid at this comparatively low temperature (500° F.), the rate of drop in temperature of the casting through its critical stage, is accurately controlled and proper malleability 20 secured during the casting operation, and at the same time, the conductivity of the molten tin is such that the mold will be cooled, or its temperature prevented from 25 rising to such a point that injury to the mold will result therefrom. Metal molds may therefore be employed and will be protected against rapid disintegration so that they may be used through long periods of time.
- 30 The conductivity of the molten tin is not however so great as to cause a too rapid cooling of the casting but will absorb sufficient heat to provide the desired retardation of drop in temperature as the metal passes 35 through its critical stage of approximately 1200° F. and give proper annealing, but sufficiently rapid to prevent the formation of graphite.
- 40 Any fluid cooling-medium may be employed which will retain sufficient heat to properly retard cooling of the casting and at the same time will have the proper degree

of heat conductivity to cool the casting and mold, but it has been found that molten tin is very efficient for the purpose and preferable.

In the drawing, a mold has been shown for the purpose of illustrating the method embodying the present invention, but it will be understood that any suitable form or construction of mold which will provide for maintaining contact of the cooling medium with the mold wall may be employed, suitable provision being made for separating the die mold parts 1 and 2 to discharge the 55 castings, as by making the parts relatively movable upon suitable guides 6 or the like and providing any suitable means, as a screw 7 for moving relatively the boxes or receptacles 8 forming the chambers 3, so that the 60 formed castings 9 may be discharged from the die or mold.

By this method the cooling of the cast metal may be very accurately controlled and time regulated to produce a uniform product, and reheating of the castings is obviated, due to this accurate and delayed cooling of the metal within the mold or die in which the casting is formed. Oxidization is also prevented as all air is excluded from the 70 casting by its inclosure within the die.

The method embodying the present invention may be modified within the scope of the appended claim, and such modifications are contemplated.

What I claim is:—

The method of casting malleable castings which consists in providing a mold, introducing molten metal into the mold to form a casting, and in maintaining a body of tin 80 in fluid state in contact with the mold walls.

In testimony whereof I affix my signature.

WILLIAM H. SMITH.